

July 15, 1930.

W. F. HAYES

1,770,520

LAMINATED BOARD

Filed June 21, 1926



FIG. 1



FIG. 2

Inventor

William F. Hayes

By *James A. Hoffman*

Attorney

## UNITED STATES PATENT OFFICE

WILLIAM F. HAYES, OF DETROIT, MICHIGAN, ASSIGNOR TO GAGNIER FIBRE PRODUCTS COMPANY, OF DETROIT, MICHIGAN

LAMINATED BOARD

Application filed June 21, 1926. Serial No. 117,480.

My invention relates to a laminated board of the type that includes a reinforced plastic composition arranged between two layers of paper or its equivalent.

It is the primary object of my invention to produce a material that is particularly adapted for use as a substitute for the composite fabric structures that are used at the present time in the construction of tops or roofs of automobiles. It is also particularly adapted for use in foundation panels in the upholstering of an automobile and for embossed panels for finishing the interior of a motor vehicle. The improved material hereinafter described is, however, capable of numerous other uses though especially designed to provide an inexpensive, but superior substitute for the materials generally used at the present time for the above specified purposes.

It is a further object of my invention to provide a laminated board that is as waterproof and moisture-proof as hard vulcanized rubber, and so tough that it can not be torn by hand. At the same time my improved material is sufficiently flexible and free from a tendency to set to permit sections that are ten feet in length to be rolled into rolls of two feet diameter, without imparting to the material within the time required for shipment the undesirable set that would prevent it from assuming its ordinary flat condition, when unrolled.

It is a further object of my invention to provide an improved board that can be nailed close to its edges to any suitable foundation structure without weakening the board and it is entirely feasible to remove any board that has been nailed in place and subsequently replace it. This is not possible in a straight fibre panel because the nail holes so weaken it that it is not advisable to replace it after it has been once removed, assuming that the panel is removed without serious injury. When my material is used the nails can safely be put in the old holes when a panel is replaced.

Other objects of the invention will appear as the description proceeds with reference to the accompanying drawing, in which,

Fig. 1 is a perspective view of my improved board, a portion of the board being broken away to show the construction thereof.

Fig. 2 is a cross sectional view of the board.

Like reference characters indicate like parts in the several views.

The body 3 of my improved board is a composition, of which the following is an example:

|                                  | Per cent |
|----------------------------------|----------|
| Asphalt or asphaltic composition | 60       |
| Rubber (pure)                    | 5        |
| Rubber (reclaimed)               | 40       |
| Inorganic filler                 | 3        |
| Rosin                            | 1        |
|                                  | 65       |

Sulphur sufficient to vulcanize the rubber compound.

I have found it advantageous and productive of very satisfactory results to use an asphaltic composition that contains about twenty per cent of stearin, though it should be understood that my invention is not restricted to the use of this composition.

Preferably, the reclaimed rubber is boot and shoe rubber though other grades may be used. The filler employed may be whiting, barium sulphate or the like.

As will be understood by those skilled in the art, the hardness of the product may be varied by increasing the filler and rosin content and by correspondingly reducing the rubber content. A flexible product is needed in foundation panels in order that it may be readily carried around the corners of the body of the car, while a harder product is desired for door panels. By varying the composition as above indicated the product having the desired characteristics may be readily produced.

The above ingredients, in the specific proportions selected, are thoroughly mixed in a rolling mill, the asphalt and rubber being first given a twenty minute run. Then the balance of the material is added, and the run continued until the mixing is complete. The batch is allowed to season for forty-eight hours and is then placed on a calendering machine, and a wire screen or other equivalent reinforcing material is embedded therein, as shown at 4 on the drawing. The compound

is then in a plastic condition. Layers 5 and 6 of paper or any other suitable material are then combined to the top and bottom of the compound and calendered to the body 3.

8 The material is then given a heat treatment of three hours duration at a temperature of 260 degrees Fahrenheit thus vulcanizing the rubber content and resulting in a product having the above stated characteristics.

10 My improved material has been found to be especially efficacious for use in automobile tops. At the present time tops are constructed of layers of chicken wire, cotton batting and top material applied separately. It has been found that by using my improved board in lieu of the materials just referred to, that a far superior top that it is practically impossible to puncture, results. And this is brought about with a reduction in cost of material of fifty per cent, and with a reduction in cost of labor of about seventy-five per cent. It has been found further that when used in top construction my improved material assumes a set form after it has been in position 25 for a comparatively long period of time, though it can be rolled for shorter periods without causing it to assume a curvilinear form, as above pointed out.

30 I have above described my invention in considerable detail. It should be understood that my invention is not restricted to such detail but that the scope thereof is to be determined from the following claims.

What I claim as my invention is:

35 1. Laminated board suitable for use for finishing the interior of a motor vehicle body characterized by the fact that it is sufficiently flexible to conform to curved surfaces of the body of said vehicle, water and moisture proof and capable of being nailed close to its edges without seriously weakening the board, consisting of surface protecting layers of paper, a wire reinforcement coextensive with said layers, and flexible cementitious material uniting said layers and reinforcement, said layers, reinforcement and material being combined by calendering.

50 2. Laminated board suitable for use for finishing the interior of a motor vehicle body characterized by the fact that it is sufficiently flexible to conform to curved surfaces of the body of said vehicle, water and moisture proof and capable of being nailed close to its edges without seriously weakening the board, consisting of surface protecting layers of paper, a wire reinforcement coextensive with said layers, and flexible cementitious material consisting of asphalt and rubber uniting said 55 layers and reinforcement, said layers, reinforcement and material being combined by calendering, and said rubber being vulcanized.

60 3. The product defined in claim 2 in which asphalt and rubber in approximately equal

proportions are utilized as cementitious material.

4. Laminated board suitable for use in finishing the interior of a motor vehicle body, characterized by the fact that it is sufficiently flexible to conform to curved surfaces of the body of said vehicle, water and moisture proof and capable of being nailed close to its edges without seriously weakening the board, consisting of surface protecting layers of paper, a wire reinforcement coextensive with said layers, and flexible cementitious material uniting said layers and reinforcement, said layers, reinforcement and material being combined by calendering, and said cementitious material being chemically changed to cause said layers, reinforcement and material to form a homogeneous structure.

70 WILLIAM F. HAYES.

85

90

95

100

105

110

115

120

125

130